

Oct. 1, 1946.

E. C. LYONS

2,408,466

MELTING MAGNESIUM METAL AND THE LIKE

Filed Nov. 9, 1944



INVENTOR.

Ellis C. Lyons

BY

Pennie, Danis, Marin, Edwards

ATTORNEYS

## UNITED STATES PATENT OFFICE

2,408,466

MELTING MAGNESIUM METAL AND  
THE LIKE

Ellis C. Lyons, Boulder City, Nev., assignor, by  
mesne assignments, to Reconstruction Finance  
Corporation, a corporation of the United States

Application November 9, 1944, Serial No. 562,722

7 Claims. (Cl. 266—33)

1

This invention relates to the melting of magnesium and magnesium base alloys, and has for its object the provision of certain improvements in the melting of magnesium and in the melting, with or without refining, of magnesium and its alloys.

Magnesium is commonly produced by the electrolysis of a fused bath of magnesium chloride or by reduction of magnesium oxide. The crude metal is characteristically contaminated with oxide, chloride or other impurities which are customarily removed by remelting and/or refining the molten metal. The refined metal is usually alloyed with other metals to impart desirable hardening and corrosion-resisting qualities thereto for structural and other mechanical and commercial uses, as, for example, in the automotive and aircraft industries. Among the many magnesium base alloys so used may be mentioned, merely by way of example, the magnesium-aluminum-zinc-manganese alloys containing 0.1 to 12% aluminum, none up to 5% zinc, none up to 3% manganese, and the balance essentially magnesium.

The melting and refining of the crude metal and the production of magnesium base alloys is customarily carried out at the plant where the magnesium is produced or in plants for refining and alloying magnesium. On the other hand, magnesium base alloys are customarily remelted and cast in foundries for manufacturing structural and other mechanical articles of the alloy.

The present invention contemplates an improved apparatus for melting and refining crude magnesium and for melting magnesium-base alloys, with or without refining. In its broad aspect, the apparatus of the invention comprises an elongated molten metal reservoir immersed in a fused salt bath, with means for introducing metal into the reservoir under conditions inhibiting oxidation, and with a valve-controlled discharge for the reservoir, the reservoir being so constructed that in operation it is filled with molten metal which flows by gravity from the point of introduction thereto to the point of discharge therefrom. In the form of the apparatus particularly adapted for use in melting and refining crude magnesium, the melted metal is held in two receptacles immersed in the fused salt bath and communicating with each other beneath the molten metal level, and in which impurities are permitted to settle out. One of the receptacles may be open to the atmosphere and the crude metal introduced into the top thereof. The other receptacle may be completely enclosed and is filled

2

with molten metal and communicates with the elongated molten metal reservoir. In the form of the apparatus particularly adapted for remelting clean and purified magnesium base alloys, the aforementioned receptacles are unnecessary for settling out impurities, and either or both may be used for introducing molten metal into the reservoir as molten metal is discharged therefrom, or other suitable means may be provided for such introduction of molten metal into the reservoir. The temperature of the fused salt bath may be controlled to maintain the molten metal in the reservoir within a predetermined temperature range.

15 The foregoing and other novel features of the invention which I believe to be patentable are set forth in the appended claims. The principles of the invention will be best understood from the following description taken in conjunction with the accompanying drawing, in which the single figure is a side elevation, partly in section and somewhat diagrammatic, of an apparatus embodying the invention.

Referring to the drawing, an insulated tank 5 holds a fused salt bath 6. The bath 6 may be heated by any convenient means but is preferably heated by one or more pairs of electrodes 7 electrically connected to a suitable source of electric energy 8 through a thermostatic control device 9 including a pyrometer 10 thermally associated with the bath.

An elongated conduit or molten metal reservoir 11 is submerged in the fused salt bath 6. The conduit is in the form of an oval coil extending from near the top to near the bottom of the bath and is appropriately supported by standards 12. The upper end of the conduit 11 communicates with the upper end of an enclosed receptacle or settling unit 13 completely submerged in the fused salt bath. A second receptacle or settling unit 14 is immersed in the fused salt bath. The receptacle 14 is open at its top, above the level of the bath, and is connected to the receptacle 13 by a conduit 15 at a level slightly below the communication of the receptacle 13 with the elongated conduit 11. The conduit 15 may advantageously slope upward from the receptacle 14 to the receptacle 13. The receptacle 14 has a depending drain 16 with a discharge valve 17 at the bottom thereof. The receptacle 13 has a similar depending drain 18 with a discharge valve 19. A heating coil 20 surrounds the lower end of each drain 16 and 18, exteriorly of the bottom of the tank 5, to prevent freezing of the metal and impurities in the drains. The lower end of the

elongated conduit 11 communicates with a discharge conduit 21 having a valve-controlled metal outlet 22. The conduit 21 and valve outlet 22 may be heated to prevent freezing of the metal.

The apparatus illustrated in the drawing is particularly adapted for magnesium refinery operation. Molten metal, solid pigs or shapes, scrap, and the like may be advantageously treated in the apparatus to separate therefrom the associated impurities such as particles of salt (cell melt), flux, oxides etc. which may contaminate the crude metal. The crude or contaminated metal to be treated, for example the pig 23 illustrated in the drawing, is introduced into the open upper end of the settling unit 14. Solid metal so introduced is melted by the heat of the fused salt bath. The impurities, being heavier than the molten magnesium metal, settle towards the bottom of the unit 14 and may be removed from time to time through the discharge valve 17 of the drain 16. Further settling of impurities takes place in the settling unit 13 and may be removed from time to time through the discharge valve 19 of the drain 18. Substantially pure metal is delivered from near the top of the settling unit 13 to the elongated conduit 11.

The fused salt bath 6 is thermostatically controlled to bring the molten metal in the elongated conduit 11 to the proper casting temperature. This can be accurately accomplished in the apparatus of the invention, since the salt bath assures uniform heating of the metal in the conduit within narrow temperature limits. Purified molten metal is withdrawn from the conduit 11, as required for casting, through the outlet 22. Casting may be carried out in sand molds, permanent molds, or the like. Except for the open charging top of the settling unit 14, the parts of the apparatus holding molten metal are completely enclosed, and the molten metal is effectively protected against oxidation or other contaminating influence. The conduit 11 is at all times completely filled with molten metal, and the contemplated flow of molten metal through the apparatus results from the action of gravity.

The elongated conduit or molten metal reservoir 11 may be made of steel, such as steel pipe. Such a metal conduit submerged in the fused salt bath has little tendency to scale, rust, pit or corrode, and hence has a long life. Similarly, the receptacles 13 and 14 and conduit 15 may be made of steel.

The fused salt bath may be heated in any appropriate manner, the electrodes and associated devices being described and illustrated merely by way of example. Thus, electric resistance units, submerged pipes through which hot gases pass, etc. may be substituted for the electrodes.

The invention while particularly adapted for treating magnesium and alloys thereof, may be employed with advantage in treating other easily oxidized metals.

I claim:

1. An apparatus of the character described comprising an elongated and substantially closed molten metal reservoir submerged in a fused bath without communication between the interior of said reservoir and the material of said bath, means operatively associated with said bath for maintaining the molten metal in the reservoir within a predetermined temperature range, a valve controlled discharge means operatively connected to one end of said reservoir, and means operatively associated with the other end of

said reservoir for introducing molten metal into the reservoir when molten metal is discharged from the reservoir.

2. An apparatus of the character described comprising an elongated and substantially closed molten metal reservoir submerged in a fused bath without communication between the interior of said reservoir and the material of said bath, a settling unit submerged in said bath and communicating near its upper end with one end of said reservoir and having a discharge in its bottom for settled matter, a valve controlled discharge means for the other end of said reservoir, and means for heating said bath.

3. An apparatus of the character described comprising an elongated and substantially closed molten metal reservoir submerged in a fused bath without communication between the interior of said reservoir and the material of said bath, a settling unit submerged in said bath and communicating near its upper end with one end of said reservoir and having a discharge in its bottom for settled matter, a valve controlled discharge means for the other end of said reservoir, said reservoir being so constructed that in operation it is filled with molten metal which flows by gravity from the end communicating with said settling unit to said discharge means, and means operatively associated with said bath for heating the same and maintaining the molten metal in said reservoir within a predetermined temperature range.

4. An apparatus of the character described comprising an elongated and substantially closed molten metal reservoir submerged in a fused bath without communication between the interior of said reservoir and the material of said bath, a settling unit submerged in said bath and communicating near its upper end with one end of said reservoir and having a discharge in its bottom for settled matter, a second settling unit open at its top and for the most part submerged in said bath and having a discharge in its bottom for settled matter, said settling units communicating with one another intermediate their ends, a valve controlled discharge means for the other end of said reservoir, and means for heating said bath.

5. An apparatus of the character described comprising an elongated and substantially closed molten metal reservoir submerged in a fused bath without communication between the interior of said reservoir and the material of said bath, a settling unit submerged in said bath and communicating near its upper end with one end of said reservoir and having a discharge in its bottom for settled matter, a second settling unit open at its top and for the most part submerged in said bath and having a discharge in its bottom for settled matter, a valve discharge means for the other end of said reservoir, said settling units communicating with one another intermediate their ends and below the communication of said reservoir with the first mentioned settling unit, said reservoir being so constructed that in operation it is filled with molten metal which flows by gravity from the end communicating with said first mentioned settling unit to said discharge means, and means for heating said bath.

6. An apparatus for melting an easily oxidized metal comprising an elongated and substantially closed molten metal reservoir submerged in a fused bath without communication between the interior of said reservoir and the material of said

5

bath, one end of said reservoir being adapted to receive molten metal melted by the heat of said bath, and a valve-controlled discharge means for the other end of said reservoir, said reservoir being so inclined that molten metal flows there-through by gravity.

7. An apparatus for melting an easily oxidized metal comprising an elongated and substantially closed molten metal reservoir submerged in a fused bath without communication between the

5

10

6

interior of said reservoir and the material of said bath, means for introducing molten metal melted by the heat of said bath into said reservoir under conditions inhibiting oxidation, and a valve-controlled discharge means for said reservoir, said reservoir being so constructed that in operation it is filled with molten metal which flows by gravity from the point of introduction thereto to the point of discharge therefrom.

ELLIS C. LYONS.